

# UNITED STATES PATENT OFFICE.

GUILLIAM H. CLAMER, OF PHILADELPHIA, PENNSYLVANIA.

## IRON-NICKEL-COPPER ALLOY.

1,016,549.

Specification of Letters Patent.

Patented Feb. 6, 1912.

No Drawing.

Application filed August 19, 1909. Serial No. 513,537.

*To all whom it may concern:*

Be it known that I, GUILLIAM H. CLAMER, a citizen of the United States, and a resident of Philadelphia, in the county of Philadelphia and State of Pennsylvania, have invented a certain new and useful Iron-Nickel-Copper Alloy, of which the following is a specification.

Objects of the present invention are first, to provide iron-copper-nickel alloys which are possessed of new uses and properties and are practically non-corrosive, which are of a low co-efficient of expansion and of great mechanical strength, which can be rolled into sheets, rods and the like, and which can be comparatively cheaply produced; and second, to provide a method or process of making a homogeneous iron-nickel-copper alloy in which on casting and cooling, no separation of metal in the form of hard nodules or otherwise occurs.

The alloy is of whitish color and it can be made within the following range of proportions by weight:

|    |        |           |
|----|--------|-----------|
| 25 | Nickel | 25 to 50% |
|    | Copper | 5 to 20%  |
|    | Iron   | 30 to 70% |

together with a small amount of impurities, such as would ordinarily exist in commercial steel, copper and nickel. Within the proportions stated the new and useful properties are attained. Carbon should not be present in amount sufficient to produce hard nodules of copper or copper mixed with nickel or of any kind.

Ordinarily, when copper and iron are melted together and cast, the perfection of the alloy depends entirely on the amount of carbon present. Pure copper and pure iron melted together in a crucible, free from carbon, will alloy in all proportions. With a small amount of carbon present, copper separates in the form of nodules and with increased amounts of carbon present, greater separation takes place, so that when the carbon content is high, for instance, as in cast iron, almost complete separation occurs. In accordance with my invention the separation of hard nodules is prevented by carefully limiting the carbon content. The strength of the alloy, however, is to a great extent regulated by the amount of carbon present. For these reasons the proportion

of carbon in the alloy cannot be definitely stated, but is fixed in any instance by having regard to the strength required of the alloy and to the carbon content that can be present without causing separation of hard nodules or otherwise. Two-tenths of one per cent. of carbon is not too much, but in mentioning this figure I do not intend to limit my patent.

For the sake of a further description, it may be stated that an alloy containing 65% iron, 25% nickel and 10% copper and  $\frac{1}{10}$  of one per cent. of carbon has the following approximate physical properties: On a test bar one-half inch in diameter and two inches between shoulders, strain per square inch in 70 pounds 96,100, limit of elasticity per square inch in pounds 51,750, elongation per cent. of original length 42%, reduction of area per cent. of original section 53.7; but the above is given without intending to limit my patent to such proportions.

To make the described alloy the ingredients thereof should be mixed, having regard to the proportions specified, and melted and cast in the usual way of preparing alloys, care being taken in melting to carefully regulate and limit the carbon content. In casting, a small amount of manganese or magnesium may, if desired, be added and when present it acts as a de-oxidizing agent. The alloy may be made directly from appropriate ore and the process of doing this forms the subject-matter of my co-pending application, serially numbered 513,538, patented August 2, 1910, No. 965,871. 90

What I claim is:

1. A homogeneous iron-nickel-copper alloy comprising nickel 25 to 50 per centum, copper 5 to 20 per centum, iron 30 to 70 per centum, and carbon and which is free from hard metallic nodules.
2. A homogeneous iron-nickel-copper alloy comprising nickel 25 to 50 per centum, copper 5 to 20 per centum, iron 30 to 70 per centum and which is free from hard metallic nodules. 100

In testimony whereof I have hereunto signed my name.

GUILLIAM H. CLAMER.

Witnesses:

M. McGARVEY.

J. CECIL BRIGHTBILL.